# EUROPEAN PATENT SPECIFICATION

(11) **EP 1 419 038 B1**
(45) Date of publication and mention of the grant of the patent: **27.12.2006**
(21) Application number: 01945073.3
(22) Date of filing: 03.05.2001
(51) Int. Cl.: B27N 7/00

(54) **METHOD FOR REDUCING FORMALDEHYDE CONTENT AND FORMALDEHYDE EMISSION FROM PARTICLEBOARD**
VERFAHREN ZUR VERMINDERUNG DES FORMALDEHYDGEHALTS UND DER FORMALDEHYDABGABE VON SPANPLATTEN
PROCEDE DE REDUCTION D'UN CONTENU FORMALDEHYDE ET D'UNE EMISSION FORMALDEHYDE A PARTIR D'UN PANNEAU DE PARTICULES

(43) Date of publication of application: 19.05.2004
(73) Proprietor: Kronospan Technical Co. Ltd., 2404 Engomi, Nicosia (CY)
(72) Inventor: FRACKOWIAK, Iwona, PL-61-546 Poznan (PL)
(74) Representative: Heselberger, Johannes
(86) International application number: PCT/EP2001/004959
(87) International publication number: WO 2002/090071

(56) References cited:
- EP-A- 0 365 708
- WO-A-92/12836
- DE-A- 19 820 833

## Description

The subject-matter of the invention is a method for producing a board and especially a method for reducing the formaldehyde content and formaldehyde emission from particleboard, to be used in the manufacturing process of particleboards, pressed in stroke and continuous-run presses, with the application of amino adhesive resins.

A method for producing a panel in accordance with the invention is known from GB 2 354 482.

Nowadays, we know of many methods for reducing the formaldehyde content and formaldehyde emission from particleboard. The major ones are:
- modification of adhesive resins, usually by the reduction of formaldehyde molar rate to urea, which most frequently leads to lessening of resin reactivity, but many times also to weaker strength of adhesive-bonded joints and their resistance to water;
- addition of formaldehyde-bonding substances. Such substances, however, may often exert negative impact on physical and mechanical properties of particleboard;
- mixing of urea-formaldehyde resins with other resins, e. g. resorcinol or phenolic ones. This in turn, is followed by substantial production cost increase;
- extension of particleboard pressing time. Followed by decrease in production capacity;
- drying of particles down to extremely low moisture content. Application is restricted by technical conditions and safety precautions due to possible ignition in drier;
- processing of particleboard with gaseous ammonia. This method requires special hermetic chambers for safety reasons;
- processing of finished particleboard with hot air in special chambers with forced intensive air exchange. This method, taking into account the actual production line capacity, would require additional special production facility in order to maintain smooth production flow;
- surface processing of finished particleboard by means of solutions of substances that come into reaction with formaldehyde. This necessitates special installation, and on the other hand there is a risk the surface quality in such particleboard would deteriorate.

As pointed out above, the presented, popular methods for reducing the formaldehyde content and formaldehyde emission from particleboard either necessitate substantial financial expenditures and operation of additional devices and installations, or some of them can also exert negative impact on production efficiency by decreasing process capacity and/or deteriorating the quality of particleboard manufactured according to such methods.

The essence of the invention for reducing the formaldehyde content and formaldehyde emission from particleboard manufactured is based on the standard method which comprises the further steps according to claim 1.

To date, the popular particleboard manufacturing methods with the application of amino resins, necessitate the particleboard cooling immediately after pressing and prior to seasoning. The cooling process takes place on rotary coolers where particleboard stays from several to a few dozen minutes, most often for the time required to decrease the particleboard internal layer temperature down to 45-60°C.

Unexpectedly, it appeared that the heat cumulated in the board or a particleboard while it is pressed, can be utilised to deepen the adhesive resin polycondensation process, which, as it should be judged, cannot be fully completed in the press due to very short board pressing cycles. The incomplete adhesive hardening can be a cause for formaldehyde splitting, consequently a rise of its content and its emission from particleboard; the emission can be long-lasting, especially in storage conditions and during implementation, which leads to considerable increase of particleboard moisture content. Short seasoning of particleboard after pressing, consistent with the invention essence, replaces to some extent the extension of particleboard pressing time. Whereas the positive influence of pressing time extension on the board's hygienic properties is already a canon in particleboard manufacturing technology. It is also known, however, that its practical application is limited due to economic aspects. On the other hand, increasing the reactivity of resins in one of the conditions for the application of technical opportunities offered by the continuous particleboard pressing system that has been introduced over the last couple of years; this additionally confirms the importance of hardening.

The to-date particleboard cooling and seasoning processes provided for test of temperature to be attained prior to seasoning, to avoid hydrolysis of adhesive-bonded joints, consequently to avoid particleboard strength diminishing. The temperature actually attained in cooling has not been controlled. For it was assumed that the lowest possible temperature was most wanted. For this reason, in modem facilities we have systems of rotary coolers instead of single devices, e.g. three rotary coolers where particleboards are successively delivered to.

The invention allows for drastic reduction of formaldehyde content and its emission from particleboard, without the need for significant changes in the actual technical and technological conditions prevailing in particleboard factories, regardless of the production line equipment, pressing process parameters, timber, and chemicals. The described above solution permits to stabilise the particleboard hygienic quality. It provides for the production of particleboard having special hygienic quality, and also for higher particleboard production efficiency due to possible application of resins features with increased molar formaldehyde to urea ratio. For tests and industrial trial technical applications of this invention revealed reduction of formaldehyde content and emission even by 70 % as compared with particleboard manufactured in conventional way, i. e. cooled after pressing. The parameters of short-time seasoning prior to cooling, i. e. temperature and time, are set depending on the expected reduction rate of formaldehyde content and emission, with due regard to characteristics of adhesive resin and application directions.

The invention subject-matter is presented below in a few practical examples illustrated with drawings. Figures 1-3 show comparative diagrams of particleboard hygienic properties, manufactured in conventional and invention method.

### Example I

To manufacture particleboard, urea-formaldehyde adhesive resin was used; urea for formaldehyde molar rate 1.0:1.5. Ammonium nitrate was the hardening agent. Particleboard pressing temperature: 205°C; at 6 s/1 mm particleboard thickness pressing time rate.

The formaldehyde content in particleboard cooled conventionally after pressing was 10.3 ing/100 mg totally dry board, whereas formaldehyde emission - some 14.9 mg/l kg totally dry board (t.d.b.). In the invention method the addition of the hardening agent to the adhesive on surface layers was reduced by 50 %.

Pursuant to the invention, the board was seasoned prior to cooling for 16 hours; whereas the temperature in the internal particleboard layer during stock-piling for brief seasoning, was 95-100°C. The formaldehyde content and emission were reduced down to 4.1 mg/100 mg totally dry board and 8.1 mg/l kg totally dry board, respectively. Thereby the formaldehyde content and emission changed positively after seasoning; whereas other particleboard properties were at the same level as in conventional production. The example is illustrated in Figure 1:
1: values for board seasoned prior to cooling;
2: values for board manufactured in conventional way (cooled after pressing).

### Example II

The 1.0 : 1.2 urea-formaldehyde adhesive resin was used for particles glue-spreading. The applied hardening agent contained known formaldehyde-bonding substances. Pressing was carried out in 218°C, at 11 s/1 mm particleboard thickness pressing time rate. The formaldehyde content in particleboard manufactured according to the conventional method amounted 4.5 mg/100 g totally dry board; whereas formaldehyde emission - 6.8 mg/l kg totally dry board. Following the brief 8 hour seasoning after pressing, and prior to cooling, in 80-85°C of particleboard internal layer, the formaldehyde content and emission where reduced down to 2.0 mg/100 mg totally dry board and 5.6 mg/l kg totally dry board, respectively. The particleboard swelling rate after soaking in water diminished by some 25 %. The hygienic quality of particleboard manufactured according to the described example is illustrated in Figure 2.

### Example III

Urea-formaldehyde-melamine resin with ammonium chloride as the hardening agent were used. The board was pressed in 185°C, at 8 s/1 mm board thickness pressing time rate. The formaldehyde content in board cooled prior to conventional seasoning amounted 8.4 mg/100 g totally dry board; whereas formaldehyde emission - 12 mg/l kg totally dry board. Following the brief 6 hour seasoning after pressing, and prior to cooling, in 90°C of board internal layer, the formaldehyde content and emission were reduced down to 5.9 mg/100 mg totally dry board and 9.7 mg/l kg totally dry board, respectively. Other properties, including water-resistance test V 100, did not change. The hygienic quality of board manufactured according to the described example is illustrated in Figure 3.

## Claims

1. A method for reducing formaldehyde content and emission from particle board from a particle board manufacturing process, in which amino adhesive resins are applied,
with the addition of hardening agents and/or the addition of formaldehyde-bonding substances;
said particle boards are pressed in continuous-run presses and cooled, wherein the particle board after pressing and prior to cooling is subjected to a brief seasoning at a temperature of between 40 and 150°C for between 8-16 hours, depending on the expected reduction rate of the formaldehyde content and emission and applied manufacturing process parameters.

2. A method according to claim 1 where a layer system step is adopted, having a base plate and a film-like layer impregnated with resin is acted upon in a pressing device with temperature and pressure on both sides in such a way that the layer system is thereby glued together.

3. A method according to claim 1 or 2, **characterized in that** the board after pressing, prior to cooling, is subjected to seasoning at a temperature of between 70 to 110°C.

## Patentansprüche

1. Ein Verfahren zum Verringern von Formaldehydgehalt und Formaldehydemission von Spanplatten bei einem Herstellungsprozess für Spanplatten, wobei Amino-Klebharze verwendet werden, mit dem Zusatz von härtenden Wirkstoffen und / oder dem Zusatz von formaldehydbindenden Substanzen; wobei die Spanplatten in kontinuierlich laufenden Pressen gepresst werden und gekühlt werden, wobei die Spanplatte nach dem Pressen und vor dem Kühlen einer kurzen Alterung bei einer Temperatur zwischen 40 und 150° Celsius für 8 bis 16 Stunden unterzogen wird, abhängig von der erwarteten Verringerungsrate des Formaldehydgehalts und Formaldehydemission und den angewandten Herstellprozessparametern.

2. Verfahren nach Anspruch 1, wobei ein Schichtsystem-Schritt eingesetzt wird, wobei auf eine Grundplatte und eine filmähnliche Schicht, die mit Harz imprägniert ist, in einer Pressvorrichtung von beiden Seiten mit Temperatur und Druck derart eingewirkt wird, dass das Schichtsystem **dadurch** zusammengeklebt wird.

3. Verfahren nach Anspruch 1 oder 2 **dadurch gekennzeichnet, dass** die Platte nach dem Pressen und vor dem Kühlen einer Alterung bei einer Temperatur zwischen 70 und 110° Celsius unterzogen wird.

## Revendications

1. Un procédé pour réduire la teneur et les émissions de formaldéhyde d'un panneau de particules issu d'un processus de fabrication de panneaux de particules dans lequel on applique des résines amino adhésives,
avec l'addition d'agents durcisseurs et/ou l'addition de substances liantes du formaldéhyde ;
lesdits panneaux de particules sont pressés dans des presses alimentées en continu et refroidis, dans lequel le panneau de particules est soumis après pressage et avant refroidissement à un bref vieillissement à une température comprise entre 40 et 150 °C pendant entre 8-16 heures, selon le taux de réduction attendu de la teneur et des émissions de formaldéhyde et des paramètres appliqués pour le processus.

2. Un procédé selon la revendication 1, où on adopte une étape de système en couche, avec une plaque de base et une couche en film imprégnée de résine est faite dessus dans un dispositif presseur avec température et pression des deux côtés d'une manière telle que le système en couche soit ainsi collé avec.

3. Un procédé selon la revendication 1 ou 2, **caractérisé en ce que** le panneau après pressage, avant refroidissement, est soumis à vieillissement à une température comprise entre 70 et 110 °C.
